

1

3,255,096

### ELECTRODEPOSITION OF NICKEL

Jack L. Towle, East Cleveland, Dale G. Block, Cleveland, and Raymond E. Bailey, Mentor, Ohio, assignors to The Harshaw Chemical Company, Cleveland, Ohio, a corporation of Ohio

No Drawing. Filed Nov. 1, 1963, Ser. No. 320,939

9 Claims. (Cl. 204—49)

This invention relates to the electrodeposition of fully bright nickel plate. More particularly, this invention relates to the use of a specific class of saturated heterocyclic compounds containing acetylenic substituents as one component of a brightener system for the electrodeposition of fully bright nickel.

According to the present invention, fully bright nickel may be deposited from any solution of nickel ions designed for plating nickel. All standard aqueous solutions designed for electroplating nickel may be used. These solutions contain at least one of the following salts: nickel sulfate, nickel chloride, nickel fluoborate and nickel sulfamate, wherein the solution is adjusted to an operating concentration of nickel. Included among the various baths useful with the present invention are (1) the various barrel plating baths generally comprising nickel sulfate and nickel chloride as the source of the nickel ion and buffer systems comprising boric acid alone or in conjunction with magnesium sulfate or ammonium chloride, (2) the all-chloride bath designed for use where a high current density is desired, comprising nickel chloride as the source of nickel ion and boric acid as the buffer, (3) the cold bath designed for use in coating objects not subject to corrosive conditions such as jewelry, comprising nickel sulfate as a source of nickel ion and boric acid and ammonium chloride comprising the buffer system, (4) the fluoborate bath comprising nickel fluoborate as the source of nickel ion and free boric acid as the buffer alone or in combination with fluoboric acid, (5) the common Watts-type bath designed for all purpose nickel plating and generally comprising nickel sulfate and nickel chloride as the source of nickel ion buffered with boric acid, and (6) the sulfamate bath.

Other ingredients are usually added to these basic constituents in order to tailor each solution for accomplishing a specific effect and result. Included among these ingredients are wetting agents such as the anionic surfactants, organic brighteners other than those of the present invention and the like.

It has been known prior to the present invention to employ various water-soluble acetylenic compounds as brighteners in nickel plating baths. Some water soluble acetylenic compounds function well as brighteners without cooperative addition agents while other water soluble acetylenic compounds function only as brighteners in conjunction with one or more cooperative addition agents.

It is generally understood by those skilled in the art that these water soluble acetylenic compounds, particularly those of relatively low molecular weight, manifest varying degrees of adsorption on the surface of the cathode being electroplated. It is also generally understood that this adsorption on the surface is desirable when the cathode is to be electroplated with a nickel deposit having full brightness.

The present invention is concerned with brightener systems comprising (a) at least one organic sulfo-oxygen

2

compound such as the aromatic sulfonamides, the aromatic sulfonimides, the aliphatic unsaturated sulfonic acids and the aromatic sulfonic acids and (b) a compound represented by the general formula

5 (I)



wherein  $n$  is an integer of from 0 to 1 inclusive, A represents a radical selected from the group consisting of  $\text{SO}_2$ ,  $=\text{C}=\text{O}$

15



and  $-\text{S}-$ , X represents an anion and R and  $\text{R}_1$  represent monovalent organic radicals. Thus the monovalent substituent represented by R can be monovalent organic radicals, examples of which are the monovalent alkyl, alkenyl, aralkyl, alkynyl, cyanoalkyl radicals and aromatic radicals and heterocyclic radicals forming part of aliphatic hydrocarbon radicals. R is only present in the quaternary salt,  $\text{R}_1$  may be a monovalent organic radical free of triple bonds such as a lower saturated hydrocarbon radical, a heterocyclic radical or hydrogen. When  $n$  is 1, Formula I represents a class of quaternary ammonium salts.

The present invention is based on the discovery that 30 the compounds as defined in Formula I may advantageously be combined with the hereinbefore mentioned sulfo-oxygen compounds to provide an excellent brightener system in baths designed for electrodepositing fully bright nickel.

35 These compounds may be employed either as unquaternized compounds or they may be employed as the quaternary ammonium salts thereof having a second acetylenic substituent or some other organic radical pendant from the in-ring nitrogen atom or they may be employed as a mixture of two or more of the compounds.

It is quite surprising and unexpected that the compounds 40 of the present invention may be used so effectively and universally as a class with the organic sulfo-oxygen compounds to provide a complete series of operative brightener systems in view of the fact it has been impossible to predict the characteristics of nickel deposits from baths containing acetylenic compounds as brighteners; the action of acetylenic compounds on the cathode surface is not 45 adequately understood. Moreover, it is especially surprising that the compounds of Formula I may be used universally as a class since the piperidino analogues of these compounds are lacking utility as brighteners because of poor brightening characteristics.

50 The compounds of the instant class are also advantageously produced in high yields and may be obtained substantially free of impurities, thus providing a low-cost source of commercially acceptable brighteners. The fact that the compounds of the present invention provide 55 a class of compounds all of which may be used as brighteners is also surprising and unexpected inasmuch as certain classes of compounds having analogous heterocyclic type unsaturated rings containing nitrogen in the nucleus including varying numbers of compounds that do not act very well as brighteners. Moreover, many of these compounds, while being extremely good brighteners, are ob-

tained only in poor yields and must be separated from a tarry mass making such compounds exorbitantly expensive. Such compounds include the quaternary ammonium heterocyclic compounds containing the quinoline, acridine and/or pyridine nuclei.

Also, it is surprising that these saturated ring compounds allow a greater range of current densities for brightness than do the analogous unsaturated ring compounds. Through the use of the saturated brighteners of the present invention it is possible to obtain a nickel deposit having a greater area of brightness for any given article of complex shape than can be obtained on nickel deposited using the unsaturated analogues.

The present invention is carried into effect merely by adding one or more of the compounds defined by Formula I with one or more of the hereinbefore mentioned organic sulfo-oxygen compounds to an aqueous solution of one or more of the required nickel salts.

The resulting solution may be employed advantageously as an electroplating bath for the deposition of fully bright nickel. When employed with Watts-type, sulfamate or fluoborate baths, the brightener systems of the present invention provide a solution which can be operated effectively at current densities ranging from 10 to 200 amps. per square ft. and preferably at current densities ranging from 25 to 100 amps. per square ft. The baths prepared according to the present invention may be operated at temperatures in the range of from 100° F. to 170° F. and preferably from 130° F. to 165° F.

In adjusting the composition of the nickel plating baths of the present invention, it is preferred that the resulting solution have a pH between 3.5 and 4.5. This pH range is however not critical; very satisfactory results are obtained from solutions having a pH value anywhere in the range of from 2 to 5.5. As in most cases, the effective concentrations for each member of the class of compounds of Formula I vary slightly and are partially dependent on the over-all bath composition and the plating conditions (temperature, current densities, etc.). The compounds defined by Formula I are effective in amounts as low as .005 g./l. and may be used advantageously in amounts up to 0.6 g./l. Preferably the bath should contain at least 0.01 g./l. of a compound defined by Formula I. Concentrations in excess of 0.6 g./l. while not being harmful provide no added advantage.

The complementing compounds (the organic sulfo-oxygen compounds) of the brightener systems of the present invention may be advantageously employed in similar amounts as the brighteners themselves. Generally it has been found, however, that the sulfo-oxygen compounds should be present in amounts ranging from about 2.0 g./l. to about 5.0 g./l. In some instances amounts as high as 40 to 50 g./l. may advantageously be used.

Using the brightener systems of the present invention, fully bright nickel may advantageously be deposited at almost any thickness. The only criteria to be used in controlling the thickness are the cost of excessive nickel and the degree of ductility demanded. Maximum ductility is obtained at the minimum thicknesses required for obtaining a fully bright plate. Using baths prepared according to the present invention, a build-up of about 0.0001 to 0.0005 inch of nickel produces a highly ductile, fully bright plate. Where a heavy plate is of primary concern, fully bright plates may be deposited to a thickness up to 0.1 inch or even higher. It is preferred, however, that the thickness of the nickel deposit be kept between 0.001 inch and 0.01 inch. A nickel deposit having a thickness in this range is fully bright and ductile and provides the protection usually required for use in most environments.

Nickel electroplating baths particularly useful in combination with the brightener systems of the present invention include the Watts-type and fluoborate type baths having increased nickel content. Such baths are designed for use with organic brighteners in general; they may

be operated at the higher current densities desirable for the effective use of the instant organic brighteners. For purposes of the present invention, the preferred Watts-type bath essentially comprises an overall nickel content ranging from 70 to 115 g./l. provided by 270 g./l. to about 450 g./l. of nickel sulfate and from about 20 g./l. to about 90 g./l. of nickel chloride with about 30 to 40 g./l. of boric acid as the buffer and the preferred fluoborate type bath essentially comprises an over-all nickel content ranging from 75 to 110 g./l. provided by about 440 g./l. of nickel fluoborate with about 30 g./l. of boric acid as the buffer.

For purposes of the present invention, boric acid is preferred as the buffer—as an additive to maintain the desired pH. However, oxalic acid, borax (sodium tetraborate), formic acid and other compounds commonly known to have utility as buffers, may be used with the baths of the present invention with no apparent undesirable effects.

Illustrative examples of wetting agents which may be employed in the baths of the present invention include a great majority of the anionic surfactants. The sulfate type may particularly be used. Included among this type are the alkyl sulfates, aralkylsulfates, alkylsulfonates, and the aralkylsulfonates.

The use of a wetting agent in baths prepared according to the present invention is optional; excellent deposits are obtained from baths having no wetting agent.

Illustrative examples of the organic sulfo-oxygen compounds to be employed as a co-brightener or cooperating addition agent of the present invention include the unsaturated aliphatic sulfonic acids, and alkali metal, ammonium, magnesium, and nickel salts thereof such as sodium vinyl sulfonate, sodium allyl sulfonate, diallyl-sulfone, Na- $\beta$ -styrene sulfonate, and the like;

The mono and binuclear sulfonic acids, and alkali metal, ammonium, magnesium, and nickel salts thereof such as benzene sulfonic acid, sodium benzene sulfonate, nickel benzene sulfonate, sodium p-toluene sulfonate, p-chlorobenzene sulfonic acid, sodium p-bromobenzene sulfonate, 1,2-dichlorobenzene sulfonic acid, sodium m-benzene disulfonate, nickel m-benzene disulfonate, 1-amino-2,5-benzene sulfonic acid, o, m, and p-sulfobenzaldehyde, sulfonated naphthalene sulfone, and the like;

The aromatic sulfonic acids, and alkali metal, ammonium, magnesium, and nickel salts thereof such as sodium benzene sulfonate, sodium p-toluene sulfonate, dichlorobenzene sulfonic acid, and the like;

The mononuclear and polynuclear aromatic sulfonamides and sulfonimides such as benzenesulfonamide, p-toluenesulfonamide, saccharin, benzylsulfonamide, N,N-dimethyl-p-toluenesulfonamide, N,N-dicarboxyethyl benzenesulfonamide, dibenzenesulfonamide, p,p'-oxy-bis(dibenzene sulfonimide, N,N-bis-(phenyl sulfonyl)-4,4'-biphenyl disulfonamide and the like;

The binuclear aromatic sulfonic acids, and alkali metal, ammonium, magnesium, and nickel salts thereof such as 2-naphthalene sulfonic acid, 1,5- or 2,7-naphthalene disulfonic acid, nickel 1,5- or 2,7-naphthalene disulfonate, naphthalene trisulfonic acid, diphenyl p,p'-disulfonic acid, 2-naphthol-3,6-disulfonic acid, 1-naphthylamine-3,6,8-trisulfonic acid, and the like;

The heterocyclic sulfonic acids, and alkali metal, ammonium, magnesium, and nickel salts thereof including thiophene sulfonic acid, 2-(4-pyridyl) ethyl sulfonic acid, 2-(2-pyridyl) ethyl sulfonic acid, and the like. Additional sulfo-oxygen compounds useful with present invention include those disclosed in U.S. Patents 2,757,133 and 2,766,284 which are incorporated herein by reference.

The examples of the compounds embraced by Formula I include the mono- and di-substituted thiazines, thiazine dioxides, piperidones, piperazines and the quaternary ammonium salts thereof including the halides, arylsulfonates, sulfates, perchlorates and the like, wherein R of Formula I may be hydrogen or a monovalent saturated hydrocar-

bon radical derived from hydrocarbons containing from 1-16 carbon atoms including methane, ethane, etc. through hexadecane; monovalent unsaturated hydrocarbon radicals derived from the mono- and polyolefins, the mono- and polyacetylenic compounds and those polyunsaturated compounds containing both double bonds and triple bonds derived from compounds having 3-10 carbon atoms including propene, butene, etc. through decene; butadiene, pentadiene, etc. through decadiene; propyne, butyne, etc. through decyne; the ethenyl, propenyl, butenyl radicals containing at least one triple bond and having from 4-10 carbon atoms; monovalent aromatic substituted aliphatic radicals derived from lower alkyl benzenes including toluene (phenyl methane), phenylethane and the like, and lower alkyl substituted benzenes including their homologues such as xylene and the like and alkyl benzenes substituted with fluorine, chlorine, bromine or the like; monovalent nitriles derived from cyanoalkyls such as  $\beta$ -cyanoethyl and the like; monovalent hydroxyalkyls derived from compounds having from 1-5 carbon atoms such as methanol (hydroxymethane), ethanol through pentanol (hydroxypentane) and the like; monovalent cycloalkyls derived from compounds having from 3-6 carbon atoms such as cyclopropane through cyclohexane and the like; and wherein  $R_1$  of Formula I represents hydrogen a lower alkyl having from 1-5 carbon atoms and a radical represented by the formula

(II)



wherein A, R and X have the same meaning as above and includes radicals derived from thiazine, thiazine dioxide, piperidone, and piperazine.

Preferably, however, R represents lower alkyl radicals having from 1-6 carbon atoms, monounsaturated alkenyl and alkynyl radicals having from 3-6 carbon atoms, benzyl and  $\beta$ -cyanoethyl and preferably R represents hydrogen.

As hereinbefore indicated when  $n$  is 1, the compounds of Formula I represent quaternary ammonium salts and X is any anion of a water soluble acid. The particular anion is not important and has little if any effect on brightening properties of these compounds. The only property the anion must have is that it be capable of forming the quaternary salt with the tertiary nitrogen of the present

compounds. Examples of useful anions represented by X include, of course, the strongly anionic single valent halogen radicals, fluoride, chloride, bromide and iodide; the single valent aryl sulfonates, benzenesulfonate and the like and the single valent peroxyhalogenates; perchlorate and the like.

Specific names of some of the compounds of Formula I include N,N-dipropargylthiazinium-1,1-dioxide bromide, N,N - dipropargylthiazinium - 1,1 - dioxide benzenesulfonate, N - allyl - N - propargylthiazinium - 1,1 - dioxide bromide, N - benzyl - N - propargylthiazinium - 1,1 - dioxide bromide, N - propargylthiazine - 1,1 - dioxide, 1,4 - bis(N - propargylthiazinium - 1,1 - dioxide bromide) - butyne - 2,1,4 - bis(N - thiazine - 1,1 - dioxide) - butyne - 2; 4-keto-1-methyl-1-propargyl piperidinium bromide, N - phenyl - N' - propargylpiperazine, N - propargyl-N-( $\beta$ -hydroxyethyl)thiazinium-1,1-dioxide bromide, N-propargyl-N-( $\beta$ -cyanoethyl) thiazinium-1,1-dioxide bromide, 4-keto-1-ethylaminoethyl-1-propargyl piperidinium bromide, N-propargyl-N-cyclohexyl thiazinium perchlorate and the like.

The preparations of the saturated ring compounds of the present invention are well known.

For instance a procedure for preparing the N-substituted thiazine 1,1-dioxide compounds of the present invention see A. C. Bellaart, Rec. Trav. Chim., 81., 156 (1962).

The saturated ring compounds (thiazine, thiazine-1,1-dioxide, etc.) themselves are well known. Effective methods for their preparation are described in the following:

The preparation of 1,4-thiazine is disclosed in an article by Cymerman-Craig et al., Chemistry and Industry, 1954, 1455; and the preparation of 1,4-piperidone is disclosed in an article by Ruzicks et al., Helv. Chim. Acta 1920, 3, 806, and the preparation of symmetrical double molecules containing two saturated rings is disclosed in an article by Ford et al., J. Am. Chem. Soc. p. 2433 (1949).

In order that those skilled in the art may better understand how the present invention can be carried into effect, the following examples are given way of illustration and not by way of limitation. All parts and percentages are by weight unless otherwise specified.

The following table includes a series of bath compositions formulated according to the present invention. Each of the compositions set forth therein is used to deposit fully bright nickel plate over a broad range of current densities and at temperatures anywhere within the hereinbefore indicated range.

TABLE

| Ex. No.   | Nickel Salts, g./l.                        | Organic Sulfo-oxygen cpd., g./l.                                       | Brightener Present Invention, g./l.                                                             | Wetting Agents, g./l.                             | Boric Acid Buffer, g./l. | pH  |
|-----------|--------------------------------------------|------------------------------------------------------------------------|-------------------------------------------------------------------------------------------------|---------------------------------------------------|--------------------------|-----|
| I.....    | Nickel chloride, 40; nickel sulfate 250.   | p,p'Oxy-bis(dibenzene-sulfonimide), 3.0.                               | N,N-dipropargylthiazinium-1,1-dioxide bromide, 0.07.                                            | Sodium 7-ethyl-2-methyl undecyl sulfate, 0.04.    | 40                       | 3.8 |
| II.....   | do.....                                    | Saccharin (Na Salt), 1.0; Bi(dibenzenesulfonamide), 3.0.               | N,N-dipropargylthiazinium-1,1-dioxide benzene sulfonate, 0.1.                                   | do.....                                           | 40                       | 3.8 |
| III.....  | do.....                                    | Saccharin (Na Salt), 2.0; Allyl sulfonate (Na Salt), 1.0.              | N-propargylthiazine-1,1-dioxide, 0.07.                                                          | do.....                                           | 40                       | 3.5 |
| IV.....   | Nickel chloride, 150; nickel sulfate, 250. | Saccharin (Na Salt), 2.0; p,p'Oxy-bis(dibenzene-sulfonimide), 2.0.     | N-allyl-N-propargylthiazinium-1,1-dioxide bromide, 0.12.                                        | do.....                                           | 40                       | 4.0 |
| V.....    | Nickel chloride, 40; nickel sulfate, 250.  | Naphthalene disulfonate, 1.0; p,p'Oxy-bis(dibenzene-sulfonimide), 3.0. | N,N-dipropargylthiazinium bromide, 0.06.                                                        | do.....                                           | 40                       | 3.8 |
| VI.....   | do.....                                    | p,p'Oxy-bis(dibenzene-sulfonimide), 3.0.                               | 4-keto-1-methyl-1-propargyl-piperidinium bromide, 0.125.                                        | do.....                                           | 40                       | 3.8 |
| VII.....  | Nickel fluoborate, 300.....                | do.....                                                                | N,N-dipropargylthiazinium-1,1-dioxide bromide, 0.28.                                            | do.....                                           | 25                       | 2.7 |
| VIII..... | Nickel chloride, 45; nickel sulfamate 450. | do.....                                                                | N-propargylpiperidone, 0.1.                                                                     | do.....                                           | 37                       | 3.5 |
| IX.....   | Nickel chloride, 300; nickel sulfate 30.   | Saccharin (Na Salt), 2; Benzene sulfonic acid, 5.                      | N-propargylthiazine-1,1-dioxide, 0.1; N-benzyl-N-propargylthiazinium-1,1-dioxide bromide, 0.12. | do.....                                           | 30                       | 3.8 |
| X.....    | Nickel chloride, 40; nickel sulfate, 250.  | Benzene sulfonic acid, 5; Benzenesulfonamide, 1.                       | N-Phenyl-N-propargyl-piperazine.                                                                | Dihexyl-ester of sodium sulfo succinic acid, 0.1. | 40                       | 3.6 |

See footnotes at end of table.

TABLE—Continued

| Ex. No. | Nickel Salts, g./l.                       | Organic Sulfo-oxygen cpd., g./l.                                                                                  | Brightener Present Invention, g./l.                                                                     | Wetting Agents, g./l.                                                                    | Boric Acid Buffer, g./l. | pH  |
|---------|-------------------------------------------|-------------------------------------------------------------------------------------------------------------------|---------------------------------------------------------------------------------------------------------|------------------------------------------------------------------------------------------|--------------------------|-----|
| XI      | Nickel chloride, 40; nickel sulfate, 250. | Saccharin (Na Salt), 2; Thiophene sulfonic acid, 0.5.                                                             | N-propargylthiazine-1,1-dioxide, 0.07. <sup>1</sup>                                                     | Dihexyl-ester of sodium sulfo succinic acid, 0.1.                                        | 40                       | 3.7 |
| XII     | do                                        | Saccharin (Na Salt), 1; Allyl sulfonate (Na Salt), 0.5; Dibenzenesulfonamide, 2.                                  | N,N-dipropargylthiazinium-1,1-dioxide perchlorate, 0.01.                                                | Sodium lauryl sulfate, 0.05.                                                             | 40                       | 4.2 |
| XIII    | do                                        | Bi(dibenzene sulfonamide), 3; Benzene sulfonic acid, 2; Benzenesulfonamide, 1; Sulfonated Naphthalene sulfone, 1. | N,N-dipropargylthiazinium dioxide bromide, 0.05. <sup>2</sup>                                           |                                                                                          | 40                       | 4.5 |
| XIV     | do                                        | Naphthalene disulfonate, 1; p,p'-Oxy-bis(dibenzene-sulfonimide), 3.                                               | 1-(N-propargylthiazinium-1,1-dioxide bromide)-4-(keto 1-propargyl-piperidinium bromide) butyne-2, 5, 0. | Dihexyl ester of sodium sulfo succinic acid, 0.02; Sodium 2-ethyl 1-hexyl sulfate, 0.02. | 40                       | 4.0 |
| XV      | do                                        | Bi(dibenzene sulfonamide), 2; Naphthalene disulfonate, 1.                                                         | 1,4-bis(N-propargylthiazinium-1,1-dioxide)butyne-2, 0.1.                                                | Sodium lauryl sulfate, 0.1.                                                              | 40                       | 5.0 |
| XVI     | Nickel fluoborate, 425                    | Benzene sulfonic acid, 5; Dibenzenesulfonamide, 2.                                                                | N-propargylthiazine-1,1-dioxide, 0.07.                                                                  | Sodium 2-ethyl 1 hexyl sulfate, 0.04.                                                    | 35                       | 2.2 |

<sup>1</sup> Bath also contained 0.01 g./l. of allyl quinaldinium bromide a well known brightener for nickel.

<sup>2</sup> Bath also contained 0.05 g./l. of ethylene cyanohydrin a well known brightener for nickel.

As a further refinement of the present invention, it has been found that the compounds embraced by Formula I, where A represents the radicals  $=C=O$  and  $=SO_2$ , may be used to provide a bath for depositing a fully bright nickel coating having excellent chromium receptivity over a wide range of current densities. Nickel plates deposited from baths containing this preferred group of compounds can be chromium plated, stripped of the chromium plate, and replated with chromium. The stripping and replating may be performed several times with no apparent decrease in chromium receptivity.

The excellent receptivity to chromium by nickel deposited from baths containing a member of this preferred class of brighteners is unusual; other nickel deposits incur a noticeable decrease in chromium receptivity after a first chromium deposit has been stripped from the nickel. Moreover, receptivity is unexpected inasmuch as a significantly lower degree of chromium receptivity is obtained using the thiazine, piperazine and piperidine analogues of these compounds. Other known compounds having excellent utility as brighteners such as N-propargylpyridinium bromide, 3-butyne-2-ol, 1,4-dicyano-butene-2, fuchsin, 3-N,N-diethylaminopropyne-1, and propargyl alcohol when tested under substantially identical conditions are not nearly so good for obtaining receptivity to chromium as are the instant thiazine dioxide and piperidone derivatives.

Good receptivity to chromium is especially significant in the automotive industry where literally millions of parts are chromium plated by mass production methods. Problems in chromium plating under these conditions are magnified because of the great number of parts being plated and because many of these parts are of different complex shapes. There is always a certain percentage of the chromium plated parts which will have defects in the surface and must be stripped and replated with chromium.

The preferred subgroup of compounds of the present invention which may be used to impart good chrome receptivity to a nickel deposit is represented by the following general formula



wherein  $n$  is a 0-1 inclusive, B represents a member of the group consisting of  $=\text{SO}_2$  and  $=\text{C}=\text{O}$ ,  $\text{R}_3$  represents a radical selected from the group consisting of methyl, ethyl, propyl, allyl, benzyl and propargyl and

25 X represents an anion selected from the group consisting of chloride, bromide, iodide, perchlorate, arylsulfonate and alkylsulfate.

Examples of specific compounds represented by the above general formula include N-propargyl thiazine-1,1-dioxide, N-propargyl-N-methyl thiazinium-1,1-dioxide 30 bromide, N-propargyl-N-ethyl thiazinium - 1,1 - dioxide bromide, N-propargyl-N-propyl thiazinium-1,1-dioxide bromide, N-propargyl-N-allyl thiazinium-1,1-dioxide bromide, N-propargyl-N-benzyl thiazinium-1,1-dioxide bromide, N,N - dipropargyl thiazinium - 1,1 - dioxide bromide, 35 4-keto-1 propargyl piperidine, 4-keto-1-methyl-1 propargylpiperidinium bromide, 4-keto-1-ethyl-1 propargylpiperidinium bromide, 4-keto-1-propyl-1 propargylpiperidinium bromide, 4-keto-1-allyl - 1 propargylpiperidinium bromide, 4-keto-1-benzyl-1-propargylpiperidinium 40 bromide and 4-keto-1,1-dipropargylpiperidinium bromide.

It has been found that very good brighteners may be made by replacing the triple bond-containing radicals of Formula I with a double bond-containing radical. Fully bright nickel deposits may be obtained from all of the nickel baths mentioned in column 1 using N-allylthiazine-1,1-dioxide. An excellent electroplating bath useful for obtaining a fully bright nickel deposit is obtained using the composition of Example X in the above table but substituting the N-phenyl-N'-propargylpiperazine with N-allylthiazine-1,1-dioxide. Generally the scope of double bond-containing brighteners is similar to that defined by the general Formula I with the triple bond substituted by the double bond.

55 While specific examples of the invention have been set forth hereinabove, it is not intended that the invention be limited solely thereto, but to include all of the variations and modifications falling within the scope of the appended claims.

What is claimed:

60 1. A bath for electrodepositing nickel comprising an aqueous acid solution of at least one nickel salt, at least one organic sulfo-oxygen compound and an effective amount of a compound of the general formula



70 wherein  $n$  is an integer from 0-1 inclusive, A is a radical selected from the group consisting of  $=\text{SO}_2$ ,  $=\text{C}=\text{O}$ ,  $-\text{S}-$  and



X represents an anion of a water soluble acid, R represents a radical selected from the group consisting of alkyl, alkenyl, alkynyl, aralkyl, alkylaminoalkyl, hydroxyalkyl and  $\beta$ -cyanoethyl groups,  $R_1$  is a radical of the group consisting of hydrogen, a lower alkyl and radical of the general formula



wherein  $n$ , A, R, and X have the same meaning.

2. The bath of claim 1 wherein A represents the  $=\text{SO}_2$  radical.

3. The bath of claim 1 wherein A represents the  $=\text{C=O}$  radical.

4. The bath of claim 1 wherein said organic sulfo-oxygen is  $p,p'$ -oxy-bis(dibenzene sulfonamide) and wherein said compound represented by the general formula is N,N-dipropargylthiazinium-1,1-dioxide bromide.

5. The bath of claim 1 wherein said organic sulfo-oxygen compound is bidibenzene sulfonamide and wherein said compound represented by the general formula is N,N-dipropargylthiazinium-1,1-dioxide benzene-sulfonate.

6. The bath of claim 1 wherein said organic sulfo-oxygen compound is sodium allyl sulfonate and wherein said compound represented by the general formula is N-propargylthiazine 1,1-dioxide.

7. The bath of claim 1 wherein said organic sulfo-oxygen compound is  $p,p'$ -oxy-bis(dibenzene sulfonimide) and wherein said compound represented by the general formula is N - allyl -  $\text{N}^+$  - propargylthiazinium-1,1-dioxide bromide.

8. The bath of claim 1 wherein said organic sulfo-oxygen compound is  $p,p'$ -oxy-bis(dibenzene sulfonimide) and wherein said compound represented by the general formula is 4-keto-1-methyl-1-propargylpiperidinium bromide.

9. The bath of claim 1 wherein said organic sulfo-oxygen compound is  $p,p'$ -oxy-bis(dibenzene sulfonimide) and wherein said compound represented by the general formula is N,N-dipropargylthiazinium-1,1-dioxide bromide.

#### References Cited by the Examiner

##### UNITED STATES PATENTS

|           |         |                       |          |
|-----------|---------|-----------------------|----------|
| 2,712,522 | 7/1955  | Kardos et al. -----   | 204-49   |
| 2,800,442 | 7/1957  | Brown -----           | 204-49   |
| 2,905,602 | 9/1959  | Kirstahler et al. --- | 204-49 X |
| 3,006,822 | 10/1961 | Todt -----            | 204-49   |
| 3,054,733 | 9/1962  | Heiling -----         | 204-49   |

20 JOHN H. MACK, Primary Examiner.

G. KAPLAN, Assistant Examiner.